

# UNITED STATES PATENT OFFICE.

WILLIAM H. ALLEN, OF DETROIT, MICHIGAN.

## RUST-PROOFING COATING FOR IRON AND STEEL.

1,290,476.

Specification of Letters Patent. Patented Jan. 7, 1919.

No Drawing.

Application filed January 8, 1917. Serial No. 141,180.

To all whom it may concern:

Be it known that I, WILLIAM H. ALLEN, a citizen of the United States, and residing at Detroit, in the county of Wayne and State 5 of Michigan, have invented a new and Improved Rust-Proofing Coating for Iron and Steel, of which the following is a specification.

This invention relates to the protection 10 of articles of iron and steel from rusting by producing surfaces of phosphates of iron, basic in character, on said articles, and its object is to provide a rust-proofing liquid which can be applied by means of a brush, 15 air spray or by dipping. While the exact formula of the basic phosphate surface is uncertain, it is thought to be  $3\text{FePO}_4 \cdot 3\text{Fe}_2\text{O}_3 \cdot 10\text{Fe}_2(\text{PO}_4)_3$ .

This invention consists of a liquid which 20 may be applied in any desired manner to the articles to be treated, and in the coating of surfaces of iron and steel with this liquid, in contradistinction to the present method of immersing the articles in a rust-proofing 25 bath consisting of a solution of acid phosphates wherein the articles remain until the proper surface on these articles is obtained, usually two hours when the bath is kept at a boiling point.

To accomplish this invention, a liquid consisting of an acid solution of a phosphate of 30 a metal is applied to the surfaces to be rust-proofed and permitted to dry. Under certain circumstances a second or third application 35 may be desirable, as when the article is covered with thick hard scales of oxid, in which case the liquid penetrates between the scales and the metal and causes the scales to fall off.

The coating liquid is prepared by mixing 40 the acid phosphates of iron, with a weak solution of phosphoric acid. While many acid phosphates are theoretically available, those of iron, zinc and manganese are alone 45 practical for anything but laboratory experiments. Where the phosphates are nor-

mally insoluble, sufficient phosphoric acid is added to produce a super- or acid-phosphate that will remain in solution. To give "body" to the liquid, an excess of acid phosphate may be added to the liquid, or a silicate or clay may be employed. If desired, the surfaces to be treated may be first heated, which insures a more intense action of the coating. The coating is left on the article 50 treated until chemical equilibrium has been established and may thereafter be brushed off or left in place until it flakes off.

The preferred composition of this coating is one hundred parts of an approximately 60 ten per cent. solution of phosphoric acid in water, to which is added approximately one per cent. by weight of ferric phosphate, which will usually so saturate the acid that it is incapable of uniting with any more 65 ferric phosphate to form soluble acid ferric phosphate. This liquid, thickened as stated above if desired, is then applied by means of a brush, air spray, trowel or by dipping. The liquid, if formed by the use of other 70 phosphates, is preferably of the same acidic strength, that is, equal to ten per cent. of phosphoric acid, and is also a saturated solution.

This liquid is particularly useful for protecting the surfaces of the steel work of buildings and bridges, before or after erection, and of railway vehicles, especially freight cars.

I claim:

1. A liquid rust-proofing to be applied to surfaces of iron and steel consisting of an approximately ten per cent. solution of phosphoric acid in water in which is dissolved approximately one per cent. by 85 weight of ferric phosphate.

2. A liquid rust-proofing to be applied to surfaces of iron and steel consisting of a solution of phosphoric acid and ferric phosphate in water, together with a thickening 90 of inert matter.

WILLIAM H. ALLEN.